



US006182407B1

(12) **United States Patent**  
**Turpin et al.**

(10) **Patent No.:** **US 6,182,407 B1**  
(b4) **Date of Patent:** **Feb. 6, 2001**

(54) **GYPSUM BOARD/INTUMESCENT MATERIAL FIRE BARRIER WALL**

(75) Inventors: **Kenneth A. Turpin**, Delta (CA); **Richard A. Versen**, Highlands Ranch, CO (US); **Bradley Burdic**, Littleton, CO (US); **Reed H. Larson**, Parker, CO (US); **Monroe W. Shumate**, Littleton, CO (US)

(73) Assignee: **Johns Manville International, Inc.**, Denver, CO (US)

(\*) Notice: Under 35 U.S.C. 154(b), the term of this patent shall be extended for 0 days.

(21) Appl. No.: **09/220,729**

(22) Filed: **Dec. 24, 1998**

(51) Int. Cl.<sup>7</sup> ..... **E04C 2/16; E04C 2/24**

(52) U.S. Cl. ..... **52/232; 52/381; 52/383; 52/784.11; 52/787.11; 52/800.12**

(58) Field of Search ..... **52/800.12, 787.11, 52/784.11, 232, 381, 383, 787.1; 42/70, 224, 703; 49/321, 501**

(56) **References Cited**

U.S. PATENT DOCUMENTS

- |             |         |                       |
|-------------|---------|-----------------------|
| Re. 34,951  | 5/1995  | Slosberg et al. .     |
| 1,159,411 * | 11/1915 | Olberg .              |
| 3,574,644   | 4/1971  | Olstowski et al. .    |
| 3,642,531   | 2/1972  | Peterson .            |
| 3,908,062 * | 9/1975  | Roberts ..... 428/282 |
| 3,945,962   | 3/1976  | Clark .               |
| 4,015,386 * | 4/1977  | Cook ..... 52/232     |
| 4,043,950   | 8/1977  | Wilmsen et al. .      |
| 4,191,675   | 3/1980  | Inagaki et al. .      |
| 4,222,926   | 9/1980  | Mizuno et al. .       |

|             |         |                              |
|-------------|---------|------------------------------|
| 4,273,879   | 6/1981  | Langer et al. .              |
| 4,282,687 * | 8/1981  | Teleskivi ..... 49/503       |
| 4,284,550   | 8/1981  | Mizuno et al. .              |
| 4,299,875 * | 11/1981 | Steele ..... 428/172         |
| 4,343,127 * | 8/1982  | Greve et al. ..... 52/785    |
| 4,563,491   | 1/1986  | Comune .                     |
| 4,571,915 * | 2/1986  | Barman ..... 52/785          |
| 4,689,256   | 8/1987  | Slosberg et al. .            |
| 4,811,538 * | 3/1989  | Lehnert et al. ..... 52/455  |
| 5,057,367   | 10/1991 | Morii et al. .               |
| 5,132,054   | 7/1992  | Stahl .                      |
| 5,175,197   | 12/1992 | Gestner et al. .             |
| 5,232,976   | 8/1993  | Horacek et al. .             |
| 5,338,349   | 8/1994  | Farrar .                     |
| 5,481,834 * | 1/1996  | Kowalczyk et al. ..... 52/64 |
| 5,498,466   | 3/1996  | Navarro et al. .             |
| 5,740,635 * | 4/1998  | Gil et al. ..... 52/79.1     |
| 5,916,077 * | 6/1999  | Tang ..... 49/501            |

\* cited by examiner

Primary Examiner—Carl D. Friedman

Assistant Examiner—Yvonne M. Horton

(74) Attorney, Agent, or Firm—John D. Lister

(57) **ABSTRACT**

A gypsum board/intumescent material fire barrier wall includes spaced apart, vertically extending metal or wooden studs with only one layer of gypsum board secured to each side of the studs to form a fire barrier wall with a wall cavity. An intumescent material barrier, that is at least coextensive in width and height with the width and height of the wall cavity, is also included in the fire barrier wall and preferably, the wall cavity contains a fibrous insulation blanket. Preferably, the spaced apart gypsum wall boards, with the intumescent material barrier, provide the fire barrier wall with two hour fire-resistive properties meeting or exceeding ASTM test standard E119 for walls and partitions.

24 Claims, 2 Drawing Sheets





FIG. 4



FIG. 5

FIG. 6  
PRIOR ART

## GYPSUM BOARD/INTUMESCENT MATERIAL FIRE BARRIER WALL

### BACKGROUND OF THE INVENTION

The present invention relates to a fire barrier wall which includes an intumescent material, and, in particular, to a two hour fire barrier wall which includes a single layer of gypsum board secured to each side of the studs within the wall and an intumescent material barrier, such as but not limited to: an intumescent coating layer containing expandable particulate graphite applied to the interior or exterior of one or both gypsum board layers; a fibrous insulation blanket, located intermediate the gypsum board layers, with an intumescent material (e.g. an intumescent coating) layer on one or both surfaces of the blanket; a woven or non-woven fibrous mat layer or layers coated with an intumescent coating containing expandable particulate graphite located on the exterior of or intermediate the gypsum board layers; or a woven or non-woven fibrous mat layer or layers with expandable particulate graphite dispersed throughout the mat located on the exterior of or intermediate the gypsum board layers or combinations thereof.

Gypsum board fire barrier walls 120, having two hour performance ratings, are currently constructed, as shown in FIG. 6. As currently constructed, these two hour fire barrier walls 120 include two layers 122 and 124 of vertically extending five-eights of an inch, type X, gypsum wallboard attached by screws to both sides of metal screw or wooden studs 126 that are spaced apart on sixteen or twenty four inch centers. The cavity defined by the interior surfaces of the inner gypsum boards and the studs is filled with an insulation material 128, such as a glass fiber or mineral wool insulation blanket. While performing as required, the use of two layers of gypsum wallboard (each wallboard layer weighing approximately 2200 pounds/thousand square feet) on both sides of the studs in these fire barrier walls adds significantly to the weight to be supported by the structural framework of a building. In addition, the time and labor involved in handling and installing two layers of gypsum wallboard on each side of the studs can add to the construction costs. Thus, there has been a need for an inexpensive, easy to install, gypsum board fire barrier wall with a two hour performance rating that does not require the use of two layers of gypsum wallboard on both sides of the studs.

Intumescent materials, such as those disclosed in U.S. Pat. No. 3,574,644; issued Apr. 13, 1971; Franciszek Olstowski et al (hereinafter "the '644 patent), can be applied (as stated in column 3, lines 1-5 of the '644 patent) in the form of a coating to "normally combustible or heat degradable materials such as wood, fiber-board, plastics, insulative ceilings or wall panels, other cellulosic building materials, or the like" to increase the flame resistance of such normally combustible or heat degradable materials. These intumescent materials form passive fire protection systems which remain inactive until subjected to heat and temperatures such as those encountered from the flames of a fire. When these passive fire protection systems are subjected to heat and temperatures, such as those encountered in a fire, these intumescent materials react, grow and expand forming a char (many times the original thickness of the coating applied) to insulate the surface to which the material is applied from the damaging effects of the heat generated by the fire.

While these materials can be quite effective as fire barriers, these intumescent materials can be corrosive to steel, stainless steel, copper, aluminum and other metals or

metal alloys, such as those commonly used in the construction industry. Thus, in applications, where these intumescent materials come in contact with metal components, e.g. metal fasteners such as screws or nails used to secure gypsum board to studs, the metal studs and other metal structural members or utilities such as piping and the like, the use of these intumescent materials can cause corrosion problems and although the disclosure of the '644 patent has been available to the construction industry for over twenty five years, gypsum board fire barrier walls are still constructed, as set forth above and shown in FIG. 6, using two layers of gypsum wallboard on both sides of the studs.

### SUMMARY OF THE INVENTION

The gypsum board/intumescent material fire barrier wall 15 of the present invention provides a solution to the need for a single layer gypsum board fire barrier wall. The gypsum board/intumescent material fire barrier wall of the present invention includes spaced apart, vertically extending metal or wooden studs with only one layer of gypsum board 20 secured to each side of the metal or wooden studs to form a fire barrier wall with a series of wall cavities. The fire barrier wall also includes an intumescent material barrier that is at least coextensive in width and height with the wall cavities and preferably, a fibrous insulation material such as but not limited to a glass fiber or mineral wool insulation within the 25 wall cavity. Preferably, the spaced apart gypsum board layers, with the intumescent material barrier, provide the fire barrier wall with two hour fire-resistant properties meeting or exceeding ASTM test standard E119 for walls and partitions.

In the first and second embodiments of the invention, the intumescent material barrier includes one or two intumescent coating layers, containing expandable particulate graphite, applied directly to the interior and/or exterior of one or both major surfaces of both of the gypsum boards. The coating layer or layers can be applied at the factory or at the job site. Preferably, the intumescent coating layers are coextensive in width and height with the major surfaces of gypsum boards to which the layers are applied so that the intumescent material layer overlays the outer sidewall surfaces of the metal or wooden studs to which the gypsum boards are affixed.

In a third embodiment of the present invention, the intumescent barrier includes one or two intumescent coating 45 layers, containing expandable particulate graphite, applied directly to the one or two major surfaces of a fibrous insulation blanket, such as a glass fiber or mineral wool insulation blanket. The intumescent coating layer or layers on the major surfaces of the fibrous insulation blanket not 50 only provide the intumescent material barrier required for the fire barrier wall, but the intumescent material layers may also enhance the product by stiffening the fibrous insulation blanket (batt) to make the blanket easier to handle and install and by encapsulating the fibers of the fibrous insulation 55 blanket to reduce the exposure of fibers. The coating layer or layers can be applied at the factory or at the job site. The intumescent barrier formed by the coated fibrous insulation is coextensive in width and height with the cavity formed by the gypsum board layers and studs and may overlay the inner 60 sidewall surfaces of the studs to which the gypsum board layers are affixed. Where the intumescent curtain or mat layers do not overlay the inner sidewall surfaces of the studs to which the gypsum board layers are affixed, the outer sidewall surfaces of the studs may be coated with an intumescent material layer.

In a fourth embodiment of the present invention, the intumescent material barrier may be a woven or non-woven

fibrous mat layer or layers with an intumescent coating containing expandable particulate graphite or a woven or non-woven fibrous mat layer or layers with expandable particulate graphite dispersed throughout the mat. When applied as a coating, the coating layer or layers can be applied at the factory or at the job site. Such an intumescent material layer or layers can be sandwiched between fibrous insulation layers within the wall cavity; applied intermediate a fibrous insulation layer and the inner major surface of one or both gypsum boards; or applied to the exterior major surface of one or both gypsum boards. The intumescent material coated or containing mat layer(s) are coextensive in width and height with the cavity formed by the gypsum board layers and studs and may overlay the outer sidewall surfaces of the studs to which the gypsum board layers are affixed. Where the intumescent material coated or containing mat layers do not overlay the outer sidewall surfaces of the studs to which the gypsum board layers are affixed, the outer sidewall surfaces of the studs may be coated with an intumescent material layer.

In a preferred embodiment of the present invention, the expandable particulate graphite containing intumescent material used in the fire barrier wall is non-acidic (has a pH greater than 7.0) and contains a corrosion inhibitor so that the corrosion of metals such as gypsum board fasteners and metal studs by the intumescent material is greatly reduced or eliminated.

#### BRIEF DESCRIPTION OF THE DRAWINGS

FIG. 1 is a partial transverse horizontal cross section through an embodiment of the gypsum board/intumescent material fire barrier wall of the present invention wherein there are intumescent material layers on or adjacent the interior or outer major surfaces of the two gypsum board layers and overlaying the metal studs.

FIG. 2 is a partial transverse horizontal cross section through an embodiment of the gypsum board/intumescent material fire barrier wall of the present invention wherein there are intumescent material layers on the outer or exposed major surfaces of the two gypsum board layers and overlaying the wooden studs.

FIG. 3 is a partial transverse horizontal cross section through an embodiment of the gypsum board/intumescent material fire barrier wall of the present invention wherein there is a fibrous insulation blanket with intumescent layers on both major surfaces of the blanket that overlay inner sidewalls of the metal studs.

FIG. 4 is a partial perspective view of the coated fibrous insulation blanket or batt used in the fire barrier wall of FIG. 3.

FIG. 5 is a partial transverse horizontal cross section through an embodiment of the gypsum board/intumescent material fire wall of the present invention wherein there is an intumescent material layer sandwiched between two insulation layers, intermediate, midway or substantially midway between the two gypsum board layers (although not shown, the studs may be wooden or metal and separately coated with the intumescent material).

FIG. 6 is a transverse horizontal cross section through a gypsum board fire wall of the prior art which is in current use.

#### DESCRIPTION OF THE PREFERRED EMBODIMENTS

As shown in FIGS. 1, 2, 3 and 5, the gypsum board/intumescent material fire barrier wall of the present invention

10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055 10060 10065 10070 10075 10080 10085 10090 10095 10100 10105 10110 10115 10120 10125 10130 10135 10140 10145 10150 10155 10160 10165 10170 10175 10180 10185 10190 10195 10200 10205 10210 10215 10220 10225 10230 10235 10240 10245 10250 10255 10260 10265 10270 10275 10280 10285 10290 10295 10300 10305 10310 10315 10320 10325 10330 10335 10340 10345 10350 10355 10360 10365 10370 10375

in FIG. 2, the intumescent material barrier includes two intumescent material layers 34 and 36, containing expandable particulate graphite, applied directly to the exposed or outer major surfaces of both of the gypsum boards. The intumescent material layers 34 and 36 may be coating layers of intumescent material, woven or non-woven fibrous mat layers coated with intumescent material, or woven or non-woven fibrous mat layers having intumescent material dispersed throughout the mat. Preferably, the fire barrier wall 20b also includes a fibrous insulation layer, such as but not limited to a glass fiber insulation blanket or batt 38, which is coextensive in height and width with the cavity defined by the studs 22 and the gypsum board layers 24 and 26 and preferably, extends into the channels of the studs 22 when channel shaped studs are used. Preferably, the intumescent material layers 34 and 36 are coextensive in width and height with the major surfaces of gypsum boards 24 and 26 to which the intumescent coating layers are applied so that the intumescent material layers overlay the outer sidewall surfaces of the wooden studs 22 to which the gypsum boards are affixed by passing screws through the intumescent material layers and the gypsum boards and into the sidewalls of the studs. With this construction the intumescent material barrier of the fire barrier wall 20b also protects the wooden studs from the effects of flames and heat. While wooden studs are shown in FIG. 2, metal studs can be used.

Preferably, the intumescent material layers 34 and 36 are coating layers of substantially uniform thickness ranging from about 15 mils to about 50 mils in thickness. These coating layers 34 and 36 may be applied in various ways, such as but not limited to, spraying the major surfaces of the gypsum boards with the intumescent coating material at the job site or at the factory or using a doctor blade on a production line to level out and set the thickness of a pool of the intumescent coating material distributed on the major surface of the gypsum board being coated prior to passing the gypsum board beneath the doctor blade. While it is preferred to coat the major surfaces of the gypsum boards in the embodiment of FIG. 2, the intumescent material layers 34 and 36 may also be a woven or non-woven fibrous mat coated with an intumescent material coating or a woven or non-woven fibrous mat, e.g. a mat formed by a wet process, with expandable particulate graphite dispersed throughout the mat. In the third embodiment 20c of the gypsum board/intumescent material fire wall barrier of the present invention, shown in FIG. 3, the intumescent barrier includes two intumescent coating layers 40 and 42, containing expandable particulate graphite, applied directly to the two major surfaces of a fibrous insulation blanket or batt 44, such as a glass fiber or mineral wool insulation blanket. The fibrous insulation blanket 44 is coextensive in height and width with the cavity defined by the studs 22 and the gypsum board layers 24 and 26 with the fibrous insulation blanket 44, preferably, projecting into the channels of the studs 22, as shown in FIG. 3, where channel shaped studs are used. Preferably, as shown in FIG. 4, the intumescent coating layers 40 and 42 are coextensive in width and height with the major surfaces of fibrous insulation blanket 44 to which the intumescent coating layers are applied so that the intumescent material layers are coextensive in height and width with the cavities defined by the gypsum boards 24 and 26 and the studs 22. Where the insulation blanket 44 projects into the channels of the studs 22 when channel shaped studs are used, the intumescent material layers overlay the inner sidewall surfaces of the studs 22 to which the gypsum boards are affixed by passing screws or other conventional mechanical fasteners through the gypsum boards and into

the sidewalls of the studs. Where the intumescent coating layers 40 and 42 do not overlay the inner sidewall surfaces of the studs to which the gypsum board layers are affixed, the outer sidewall surfaces of the studs may be coated with an intumescent material layer. The studs can be either metal or wooden studs.

Preferably, the intumescent material layers 40 and 42 are coating layers of substantially uniform thickness ranging from about 15 mils to about 50 mils in thickness. These coating layers 40 and 42 on the fibrous insulation blanket 44 of FIG. 4 may be applied in various ways, such as but not limited to, spraying the major surfaces of the fibrous insulation blanket 44 with the intumescent coating material at the job site or at the factory or using a doctor blade on a production line to level out and set the thickness of a pool of the intumescent coating material distributed on the major surface of the fibrous insulation blanket being coated prior to passing the fibrous insulation blanket beneath the doctor blade. The intumescent coating layers 40 and 42 on the major surfaces of the fibrous insulation blanket 44 not only provide the intumescent material barrier required for the fire barrier wall 20c, but the intumescent material layers 40 and 42 may also enhance the product by stiffening the fibrous insulation blanket (batt) to make the blanket easier to handle and install and by encapsulating the fibers of the fibrous insulation blanket to reduce the exposure of fibers. While an intumescent coating layer on each major surface of the fibrous insulation blanket is preferred, a coating layer may be applied to only one major surface of the blanket.

In the fourth embodiment 20d of the gypsum board/intumescent material fire barrier wall of the present invention shown in FIG. 5, the intumescent material barrier may be an intumescent material mat layer 48 including a fibrous woven or non-woven mat coated with an intumescent coating containing expandable particulate graphite or a woven or non-woven fibrous mat, e.g. a glass fiber mat of randomly oriented fibers made by a conventional wet process, with expandable particulate graphite dispersed throughout the mat. Preferably, the intumescent material mat layer 48 is sandwiched between fibrous insulation layers 50 and 52 as shown in FIG. 5. However, intumescent material mat layers 48 can be applied directly to the interior or exterior major surfaces of the gypsum boards 24 and 26 as discussed above in connection with FIGS. 1 and 2, or two such intumescent material mat layers 48 can be applied intermediate a fibrous insulation layer and the inner major surfaces of the gypsum board layers 24 and 26 instead of using a coated fibrous insulation blanket as in the embodiment of FIG. 3.

The intumescent material mat layer 48 is coextensive in width and height with the cavity formed by the gypsum board layers 24 and 26 and the studs 22 and, where channel shaped studs are used, may extend into the channels of the studs to which the gypsum board layers are affixed. Where the intumescent material mat layers do not extend into the channels of the studs to which the gypsum board layers are affixed, the outer sidewall surfaces of the studs may be coated with an intumescent material layer.

The preferred intumescent material used in the two hour fire wall of the present invention includes expandable particulate graphite. This preferred intumescent material may be: a coating material containing expandable particulate graphite that is applied directly to major surfaces of the gypsum board; a fibrous insulation blanket, e.g. a glass fiber insulation blanket or batt, coated with a coating material containing expandable particulate graphite; a curtain member or mat, e.g. a wet laid glass fiber mat, coated with a coating material containing expandable particulate graphite;

or a curtain member or mat, e.g. a wet laid glass fiber mat, with expandable particulate graphite dispersed throughout the mat.

Expandable particulate graphite, as used in the preferred intumescent material of the present invention, is prepared from particulate, naturally occurring crystalline flake graphite or crystalline lump graphite, that has been acid treated to make the particulate graphite intumescent. Preferably, the particulate is naturally occurring crystalline flake graphite. In the production of a preferred form of the expandable particulate graphite, it is believed that the treatment of the crystalline flake graphite or crystalline lump graphite with concentrated sulfuric acid in the presence of an oxidizing agent, such as nitric acid, forms the compound graphite sulfate which exfoliates and expands when exposed to a flame or any other heat source having a temperature of about 150° C. or greater. When exposed to temperatures of 150° C. or greater, the expandable particulate graphite used in the intumescent material of the present invention expands from about 20 to about 200 times its unexpanded volume to fill voids and cavities, form firestopping layers, and otherwise form firestopping barriers.

One method of preparing the naturally occurring crystalline flake graphite or crystalline lump graphite to make the particulate graphite expandable is disclosed in U.S. Pat. No. 3,574,644; issued Apr. 13, 1971; Franciszek Olstowski et al (the disclosure of U.S. Pat. No. 3,574,644, is hereby incorporated herein by reference in its entirety). As set forth in the '644 patent, the method includes contacting the particulate graphite, at about room temperature, (1) with a mixture of from about 8 to about 98 weight percent concentrated sulfuric acid (at least about 90 weight percent H<sub>2</sub>SO<sub>4</sub>) and from about 92 to about 2 weight percent concentrated nitric acid (at least about 60 weight percent HNO<sub>3</sub>), or (2) with fuming nitric acid, or (3) with fuming sulfuric acid, or (4) with concentrated sulfuric acid (at least about 90 weight percent H<sub>2</sub>SO<sub>4</sub>) or concentrated nitric acid (at least 60 weight percent HNO<sub>3</sub>), plus at least about 2 weight percent of a solid inorganic oxidizer, such as, for example, manganese dioxide, potassium permanganate, potassium chlorate, chromium trioxide, and the like. The resulting mix components usually are employed on a weight proportion basis from about 0.2-2/1 (acid member/graphite). These are maintained in contact for at least about one minute, although a contact time of hours or days is not detrimental. The acid treated graphite particulate, now expandable, is separated from any excess acid, water washed and dried.

In the preferred intumescent material used in the present invention, any residual acid or acid components are removed from the expandable particulate graphite, preferably by washing the expandable particulate graphite with water, to increase the pH of the expandable particulate graphite to about 7.0 and eliminate or essentially eliminate potential corrosive agents from the expandable particulate graphite. If the residual acid or acid components are not removed from the expandable particulate graphite prior to introducing the expandable particulate graphite into and mixing the expandable particulate graphite with the carrier, the corrosion inhibitor (e.g. sodium hexa meta phosphate) in the carrier can change the acid residue or acid components on the expandable particulate graphite into salt so that these corrosive agent is still present in the intumescent material in some form.

In the preferred method of making the intumescent material used in the present invention, after the expandable particulate graphite has been thoroughly washed, the expandable particulate graphite is added to a liquid carrier,

such as a coating forming carrier, containing a corrosion inhibitor and, in most embodiments, a filler. As mentioned above, the preferred intumescent material used in the fire barrier wall of the present invention (the carrier with the expandable particulate graphite, the corrosion inhibitor and filler, if used) has a pH greater than 7.0, preferably between about 7.5 and about 10.0 and most preferably, between about 8.0 and about 8.5, to reduce the corrosive properties of the intumescent material with respect to most metals used in the construction industry, except aluminum, (e.g. steel, stainless steel, and copper) and to provide a chemically conducive environment for the corrosion inhibitor to form a protective layer on any metal with which the intumescent material comes in contact to prevent or greatly reduce corrosion. If the pH of the liquid carrier, to which the expandable particulate graphite is to be added, is not within the ranges set forth above, a pH enhancer (basic material), such as but not limited to ammonium hydroxide or other hydroxides, can be added directly to the carrier or applied to the washed expandable particulate graphite, prior to introducing the expandable particulate graphite into the carrier, to bring the intumescent material of the present invention within the required pH range.

Preferably, the corrosion inhibitor, in or added to the carrier, is sodium hexa meta phosphate (which appears to work the best), sodium meta phosphate, sodium silicate or other sodium based phosphate compounds. At the pH levels used in the intumescent material of the present invention (i.e. above 7.0, preferably between about 7.5 and about 10.0 and most preferably, between about 8.0 and about 8.5) the phosphate or silicate precipitates out of the carrier to form a phosphate or silicate corrosion inhibiting layer on a metal surface that prevents oxygen from diffusing onto the metal surface. The corrosion inhibitors, listed above, function to form a protective layer when the pH is above 7.0. However, the corrosion inhibitors listed above, function better to form a protective layer when the pH of the intumescent material is between 7.5 and 10.0 and function best to form a protective layer when the pH level of the intumescent material is between about 8.0 and 8.5. Preferably, the corrosion inhibiting properties of the intumescent material of the present invention meet or exceed the following standards, ASTM C665.

The corrosion inhibitor can be introduced into the carrier in dry or solution form and is present in the carrier in sufficient quantities to form a protective layer on any metal brought into contact with the intumescent material, such as metal screws, nails or other metallic mechanical fasteners, metal studs, piping and other utilities, etc., to prevent or inhibit corrosion. For example, a carrier, such as an acrylic latex carrier, including between about 200 parts per million and about 10,000 parts per million sodium hexa meta phosphate and having a pH between about 7.5 and about 10.0 has been found to produce a satisfactory corrosion inhibiting layer and a carrier, such as an acrylic latex carrier, including between about 1,000 parts per million and about 2,000 parts per million sodium hexa meta phosphate and having a pH between about 8.0 and about 8.5 has been found to produce a satisfactory corrosion inhibiting layer.

The liquid carrier used in the preferred intumescent material of the present invention is a coating forming carrier, such as but not limited to, acrylic latexes, vinyl latexes, butadiene-styrene latexes, alkyl paints, epoxy solutions, urethane solutions, varnishes, lacquers. The viscosity of the carrier can be adjusted, as required, for type of coating or spray application being used, e.g. by regulating the amount of water or solvent added to the carrier.

To reduce the cost of the intumescent material of the present invention, many of the embodiments of the present invention include a filler, preferably an inorganic filler. For example, fillers which can be used in the intumescent material of the present invention include, but are not limited to, calcium carbonate, magnesium carbonate, dolomite and various clays commonly used as fillers.

In embodiments of the preferred intumescent material for the fire barrier wall of the present invention which include a liquid carrier and the expandable particulate graphite, but no fillers, the intumescent material is between about 40 and about 90 weight percent liquid carrier and between about 10 and 60 weight percent expandable particulate graphite. In embodiments of the intumescent material of the present invention which include fillers, the liquid carrier is between about 20 and about 60 weight percent of the intumescent material; the expandable particulate graphite is between about 10 and about 30 weight percent of the intumescent material; and the filler is between about 10 and about 50 weight percent of the intumescent material. In the preferred embodiments of the present invention which include fillers, the liquid carrier is between about 35 and about 55 weight percent of the intumescent material; the expandable particulate graphite is between about 10 and about 20 weight percent of the intumescent material; and the filler is between about 25 and about 45 weight percent of the intumescent material.

In describing the invention, certain embodiments have been used to illustrate the invention and the practices thereof. However, the invention is not limited to these specific embodiments as other embodiments and modifications within the spirit of the invention will readily occur to those skilled in the art on reading this specification. Thus, the invention is not intended to be limited to the specific embodiments disclosed, but is to be limited only by the claims appended hereto.

What is claimed is:

1. A gypsum board/intumescent material fire barrier wall comprising:

spaced apart, vertically extending studs; each of the studs having a first side and a second side; a first gypsum board layer and a second gypsum board layer; the first gypsum board layer secured to the first side of the studs and the second gypsum board layer secured to the second side of the studs and forming a fire barrier wall with a wall cavity having a width and a height that is defined, in part, by the studs and opposed major surfaces of the first and second gypsum board layers; the wall cavity having only one gypsum board layer on each side of the studs; and an intumescent material barrier, the intumescent material barrier being coextensive in width and height with the width and height of the wall cavity.

2. The gypsum board/intumescent material fire barrier wall according to claim 1, wherein: the intumescent material barrier is a coating containing expandable particulate graphite applied to the opposed major surfaces of the first and second gypsum boards; and the first and second gypsum board layers and the intumescent material barrier provide the fire barrier wall with two hour fire-resistive properties meeting or exceeding ASTM test standard E119 for walls and partitions.

3. The gypsum board/intumescent material fire barrier wall according to claim 2, wherein: the intumescent coating material has a pH greater than 7.0 and a corrosion inhibitor.

4. The gypsum board/intumescent material fire barrier wall according to claim 2, including: a layer of fibrous

insulation intermediate the opposed major surfaces of the first and second gypsum board layers and coextensive in width and height with the width and height of the wall cavity.

5. The gypsum board/intumescent material fire barrier wall according to claim 4, wherein: the intumescent coating material has a pH between about 7.5 and about 10.0 and a corrosion inhibitor; a liquid carrier is between about 40 and about 90 weight percent of the intumescent material as applied; and the expandable particulate graphite is between about 10 and about 60 weight percent of the intumescent material as applied.

6. The gypsum board/intumescent material fire barrier wall according to claim 4, wherein: the intumescent coating material has a pH between about 8.0 and about 8.5 and a corrosion inhibitor; a liquid carrier is between about 20 and about 60 weight percent of the intumescent material as applied; and the expandable particulate graphite is expandable flake graphite and is between about 10 and about 30 weight percent of the intumescent material as applied; and an inorganic filler is between about 10 and about 50 weight percent of the intumescent material as applied.

7. The gypsum board/intumescent material fire barrier wall according to claim 1, wherein: the intumescent material barrier is a coating containing expandable particulate graphite applied to the outer major surfaces of the first and second gypsum board layers; and the first and second gypsum board layers and the intumescent material barrier provide the fire barrier wall with two hour fire-resistive properties meeting or exceeding ASTM test standard E119 for walls and partitions.

8. The gypsum board/intumescent material fire barrier wall according to claim 7, wherein: the intumescent coating material has a pH greater than 7.0 and a corrosion inhibitor.

9. The gypsum board/intumescent material fire barrier wall according to claim 8, including: a layer of fibrous insulation intermediate the opposed major surfaces of the first and second gypsum board layers and coextensive in width and height with the width and height of the wall cavity.

10. The gypsum board/intumescent material fire barrier wall according to claim 9, wherein: the intumescent coating material has a pH between about 7.5 and about 10.0 and a corrosion inhibitor; a liquid carrier is between about 40 and about 90 weight percent of the intumescent material as applied; and the expandable particulate graphite is between about 10 and about 60 weight percent of the intumescent material as applied.

11. The gypsum board/intumescent material fire barrier wall according to claim 4, wherein: the intumescent coating material has a pH between about 8.0 and about 8.5 and a corrosion inhibitor; a liquid carrier is between about 20 and about 60 weight percent of the intumescent material as applied; and the expandable particulate graphite is expandable flake graphite and is between about 10 and about 30 weight percent of the intumescent material as applied; and an inorganic filler is between about 10 and about 50 weight percent of the intumescent material as applied.

12. The gypsum board/intumescent material fire barrier wall according to claim 1, wherein: the intumescent material barrier is a fibrous insulation blanket with a coating layer of an intumescent coating material containing expandable particulate graphite on at least one major surface of the fibrous insulation blanket; the fibrous insulation blanket is within the wall cavity intermediate the gypsum board layers; and the first and second gypsum board layers and the intumescent material barrier provide the fire barrier wall with two

## 11

hour fire-resistive properties meeting or exceeding ASTM test standard E119 for walls and partitions.

13. The gypsum board/intumescent material fire barrier wall according to claim 12, wherein: the intumescent coating material containing expandable particulate graphite is on both major surfaces of the fibrous insulation blanket.

14. The gypsum board/intumescent material fire barrier wall according to claim 12, wherein: the intumescent coating material has a pH between about 7.5 and about 10.0 and a corrosion inhibitor; a liquid carrier is between about 40 and about 90 weight percent of the intumescent material as applied; and the expandable particulate graphite is between about 10 and about 60 weight percent of the intumescent material as applied.

15. The gypsum board/intumescent material fire barrier wall according to claim 12, wherein: the intumescent coating material has a pH between about 8.0 and about 8.5 and a corrosion inhibitor; a liquid carrier is between about 20 and about 60 weight percent of the intumescent material as applied; and the expandable particulate graphite is expandable flake graphite and is between about 10 and about 30 weight percent of the intumescent material as applied; and an inorganic filler is between about 10 and about 50 weight percent of the intumescent material as applied.

16. The gypsum board/intumescent material fire barrier wall according to claim 1, wherein: the intumescent material barrier is a mat with a coating layer of an intumescent coating material containing expandable particulate graphite on at least one of its major surfaces; the mat is coextensive in width and height with the wall cavity; and the first and second gypsum board layers and the intumescent material barrier provide the fire barrier wall with two hour fire-resistive properties meeting or exceeding ASTM test standard E119 for walls and partitions.

17. The gypsum board/intumescent material fire barrier wall according to claim 16, wherein: the mat is intermediate the gypsum board layers.

18. The gypsum board/intumescent material fire barrier wall according to claim 17, wherein: the intumescent coating material has a pH greater than 7.0 and a corrosion inhibitor.

## 12

19. The gypsum board/intumescent material fire barrier wall according to claim 17, including: a layer of fibrous insulation intermediate the opposed major surfaces of the first and second gypsum boards and coextensive in width and height with the width and height of the wall cavity.

20. The gypsum board/intumescent material fire barrier wall according to claim 19, wherein: the intumescent coating material has a pH between about 7.5 and about 10.0 and a corrosion inhibitor; a liquid carrier is between about 40 and about 90 weight percent of the intumescent material as applied; and the expandable particulate graphite is between about 10 and about 60 weight percent of the intumescent material as applied.

21. The gypsum board/intumescent material fire barrier wall according to claim 19, wherein: the intumescent coating material has a pH between about 8.0 and about 8.5 and a corrosion inhibitor; a liquid carrier is between about 20 and about 60 weight percent of the intumescent material as applied; and the expandable particulate graphite is expandable flake graphite and is between about 10 and about 30 weight percent of the intumescent material as applied; and an inorganic filler is between about 10 and about 50 weight percent of the intumescent material as applied.

22. The gypsum board/intumescent material fire barrier wall according to claim 1, wherein: the intumescent material barrier is a fibrous mat containing expandable particulate graphite; the fibrous mat is at least coextensive in width and height with the width and height of the wall cavity; and the first and second gypsum board layers and the intumescent material barrier provide the fire barrier wall with two hour fire-resistive properties meeting or exceeding ASTM test standard E119 for walls and partitions.

23. The gypsum board/intumescent material fire wall barrier according to claim 22, wherein: the fibrous mat is intermediate the opposed major surfaces of the first and second gypsum board layers.

24. The gypsum board/intumescent material fire barrier wall according to claim 23, wherein: the expandable particulate graphite is flake graphite and the expandable particulate graphite is dispersed throughout the fibrous mat.

\* \* \* \* \*